

# UNITED STATES PATENT OFFICE.

ELI F. BURCH, OF LAUREL SPRINGS, NEW JERSEY, ASSIGNOR TO CREW LEVICK COMPANY, A CORPORATION OF PENNSYLVANIA.

## PROCESS OF MAKING PLASTIC LUBRICATING COMPOUNDS.

1,238,101.

Specification of Letters Patent. Patented Aug. 28, 1917.

No Drawing.

Application filed June 16, 1916. Serial No. 103,929.

To all whom it may concern:

Be it known that I, ELI F. BURCH, a citizen of the United States, residing at Laurel Springs, in the county of Camden and State 5 of New Jersey, have invented certain new and useful Improvements in Processes of Making Plastic Lubricating Compounds, of which the following is a full, clear, and exact specification.

10 This invention relates to a process of making lubricating compounds, and its object is to produce a lubricating compound which shall be insoluble in water, possess great affinity for metallic surfaces, be of thick 15 or semi-solid consistency, plastic and very unctuous, and shall also be stable and maintain its consistency over a wide range of temperature.

Prior to my process, so far as I am aware, 20 it has not been practicable to produce a semi-solid lubricating compound composed largely of asphaltic oils because of the tendency of the oil to become stringy, or to coagulate, as the result of the thickening 25 process, and also because of the lack of plasticity in the thickened oil.

In carrying out my invention, I take, as an example, approximately 60% of an asphaltic oil, such as heavy engine oil or black 30 oil or other benzene soluble asphaltic oil; and approximately 40% of a petroleum oil of the paraffin series, such as an oil comprising mainly or largely dodecane. These oils are mixed in a still at a temperature of 35 approximately 200° F., in order to secure a thorough mixture. The mixture is then agitated by blowing air therethrough by any suitable means, such as a perforated pipe, and at the same time the temperature is 40 raised to approximately 400° F. to 450° F. and maintained at such temperature during the necessary blowing operation. During the blowing operation, a considerable quantity of water, increasing with increase in 45 heat, will pass over as distillate, but such oil distillate as may simultaneously occur will be negligible. As the blowing is continued, the mixture will be reduced to thicker consistency, and finally to a semi- 50 fluid or grease consistency; for example, about as thick as hard vaseline.

The resultant product possesses a high degree of plasticity without stringiness or coagulation, and by reason thereof, as well as 55 because of its lubricating characteristics

and its insolubility in water, it is especially useful as a lubricant for the bearing surfaces of hydraulic machinery, or other parts which are often submerged or subjected to the action of flowing water.

Having thus described my invention, I declare that what I claim as new and desire to secure by Letters Patent is:—

1. The process of preparing a lubricant, which consists in mixing an asphaltic oil 65 and a paraffin oil, the latter having approximately the physical properties of dodecane, then heating the mixture to a temperature of approximately 400° F. to 450° F. and blowing air through the heated mixture. 70

2. The process of preparing a lubricant which consists in mixing an asphaltic oil and a paraffin oil having approximately the physical properties of dodecane, then heating the mixture to a temperature of approximately 400° F. to 450° F. and agitating the 75 same in the presence of air.

3. The process of preparing a lubricant which consists in mixing an asphaltic oil and a paraffin oil, the latter having approximately 80 the physical properties of dodecane, then heating the mixture to a thickening temperature, and simultaneously agitating the same in the presence of air.

4. The process of treating a liquid lubricant of mixed asphaltic oil and paraffin oil to make it suitable for use in contact with water which consists in heating it and blowing air through the heated mixture. 85

5. The process of preparing a lubricant 90 which consists in mixing a liquid asphaltic oil and a liquid paraffin oil, heating the mixture, and blowing air through it until it is reduced to a thick plastic consistency and is homogeneous and stable. 95

6. The process of preparing a lubricant which consists in mixing a liquid asphaltic oil and a liquid paraffin oil, heating the mixture, and blowing air through it, thereby 100 distilling off water and reducing it to a thick plastic mass of homogeneous and stable character.

7. The process of preparing a lubricant which consists in mixing asphaltic oil and paraffin oil, heating moderately to facilitate 105 their thorough mixture, then heating to a higher temperature and blowing air through the mixture, the proportion of the ingredients and the temperatures and the duration of the last mentioned stage of treatment be- 110

ing such as to give a resulting lubricant of thick plastic consistency, insoluble in water, possessing great affinity for metallic surfaces, stable, and homogeneous.

- 5 8. The process of preparing a lubricant which consists in mixing asphaltic oil and paraffin oil, heating the mixture, and blowing air therethrough, the proportion of the ingredients and the temperatures and the  
10 duration of the last mentioned stage of treatment being such as to give a resulting

lubricant of thick plastic consistency, insoluble in water, possessing great affinity for metallic surfaces, stable, and homogeneous.

In testimony whereof I affix my signature, in presence of two witnesses.

ELI F. BURCH.

Witnesses:

WILLIAM F. PALMER,  
C. V. EDWARDS.